

## UNITED STATES PATENT OFFICE

2,081,357

## METHOD OF IMPROVING GASOLINE

Vladimir Ipatieff, Chicago, Ill., assigner to Universal Oil Products Company, Chicago, Ill., a corporation of Delaware

No Drawing. Application July 5, 1932, Serial No. 620,992. Renewed July 25, 1935

4 Claims. (Cl. 196—10)

This invention refers more particularly to the manufacture of hydrocarbons of an aromatic or cyclic character suitable for use as high anti-knock blending material in motor fuel, such as gasoline.

In a more specific sense the invention relates to the more efficient utilization of the gaseous by-products of cracking so that they are employed to increase the yield, the anti-knocking character and the stability of cracked gasolines. While the process is of special value in its application to cracking processes, its use is also of commercial advantage in balancing the overall operations in the refining of crude petroleums.

Owing to the adoption of high compression ratios in automobile engines to increase their thermodynamic efficiency a demand has been made upon the petroleum refining and other industries which furnish hydrocarbon motor fuels, for fuels of a high anti-knocking or slow-burning character. The cracking process which generally produces both unsaturated hydrocarbons and cyclic hydrocarbons due to the dehydrogenating character of the decomposition reactions is employed quite generally to meet the demand for a high anti-knock motor fuel. However, complete control of the proportion of aromatics to olefins is not always possible as the character of charging oils varies with the type of crude oil from which they are produced and when intensive cracking conditions are employed in an effort to increase the amount of aromatics and hence the anti-knock value, undesirably large losses in gas and coke are encountered and frequently the amount of olefins, particularly those of a highly unsaturated and unstable character, increases roughly in proportion to the increase in aromatics. As a general rule the percentage of olefins in the gaseous products from cracking operations also increases in proportion to the intensity of cracking conditions.

The present process comprises as one of its steps the utilization of the olefinic content of gases from cracking operations, these olefins being caused to unite with aromatic compounds so that hydrocarbons of high anti-knock value are produced. Other objects and advantages will become evident as the description of the invention proceeds.

In one specific embodiment the invention com-

prises subjecting gases from cracking to temperatures above 900° C., under sub-atmospheric pressures for periods of time less than 0.1 second to increase the olefinic content thereof and then causing the olefins in the highly olefinic gas mixture to combine with aromatic hydrocarbons in the presence of sulphuric acid at normal or sub-atmospheric temperatures to produce aromatic hydrocarbon derivatives of high anti-knock value.

In a further specific embodiment, hydrocarbon gas mixtures from cracking or other sources containing substantial percentages of hydrocarbons of more than one carbon atom are subjected to temperatures in excess of 900° C. at sub-atmospheric pressures for times under 0.1 second and the olefins in the gas are then caused to combine with aromatic hydrocarbons in the presence of sulphuric acid, the aromatic hydrocarbons being present in hydrocarbon mixtures of approximate motor fuel boiling range.

The first step of the present process wherein unsaturated hydrocarbons such as acetylene, ethylene, propylene, butylenes, amylenes, etc., are produced by pyrolytic treatment of hydrocarbon gas mixtures differs from previously employed processes principally in the use of sub-atmospheric pressures of the order of 50 mm. of mercury absolute in contrast to atmospheric or superatmospheric pressures and the use of extremely low time factors of the order of 0.01 second or lower in most instances, the effect of the combined reduction in pressure and time of treatment serving to arrest the reactions of decomposition at a point corresponding to the initial stage of decomposition of the hydrocarbons concerned so that subsequent condensation and rearrangements of unstable radicals into compounds of a cyclic character is substantially prevented. Previous pyrolytic processes employed upon hydrocarbon gas mixtures similar to those to which the first step of the present process may be applied have produced relatively low yields of the olefinic hydrocarbons, sometimes only a fraction of 1% while under the customarily used conditions of temperature, pressure and time the best yields of olefins seldom exceed 15 to 20%. The first step of the present process makes possible the production of greatly improved yields of olefinic hydrocarbons as will

be shown in the examples to be subsequently given.

Table 1 contains significant data obtained in treating gases from a widely used commercial cracking process by the first step of the process of the present invention, and shows the yields of different unsaturated hydrocarbons obtained at different temperatures and low contact times.

The original gas mixture had the following composition:

|                 | Volume percent |
|-----------------|----------------|
| Acetylene       | 0.4            |
| Ethylene        | 4.6            |
| Propylene       | 5.4            |
| 1-Butene        | 2.9            |
| 1,3 Butadiene   | 4.3            |
| Methane         | 26.6           |
| Ethane          | 21.1           |
| Propane         | 16.3           |
| n-Butane        | 1.5            |
| i-Butane        | 0.8            |
| n-Pentane       | 1.9            |
| i-Pentane       | 1.7            |
| Hydrogen        | 5.8            |
| Carbon monoxide | 0.5            |
| Carbon dioxide  | 1.5            |
| Nitrogen        | 4.7            |
|                 | 100.0          |

The pressure employed in the runs which furnished the data given in the table was 50 mm. of mercury absolute.

Table I

| Temperature,<br>°C. | Maximum liters of hydrocarbons<br>from 100 liters of gas |          |           | Contact time<br>in seconds at<br>maximum<br>yield |
|---------------------|----------------------------------------------------------|----------|-----------|---------------------------------------------------|
|                     | Propylene                                                | Ethylene | Acetylene |                                                   |
| 1400                | 0.96                                                     | 10.5     | 43.0      | 0.0050                                            |
| 1300                | 2.4                                                      | 24.8     | 26.0      | 0.0058                                            |
| 1200                | 2.8                                                      | 31.5     | 19.0      | 0.0065                                            |
| 1100                | 7.4                                                      | 41.8     | 9.0       | 0.0074                                            |
| 1000                | 10.9                                                     | 29.6     | 2.0       | 0.0085                                            |

Consideration of the above data indicates that a temperature of 1100° C. produced the maximum yield of ethylene and that increasing or decreasing temperature decreased the yield. The yield of propylene representing olefins of higher molecular weight than ethylene increased with decreasing temperature while the yield of acetylene decreased markedly with decreasing temperature, reaching a negligible value at 1000° C. The time factors employed will be seen to be extremely small in comparison to time factors frequently employed in the pyrolytic treatment of hydrocarbon gas mixtures for the same objects. The use of the low time factor corresponds to a high yield of desired products for a given size of equipment.

It will be seen also that since the relative proportions of acetylene, ethylene and propylene vary with the temperature of treatment under approximately equivalent conditions of time factor that some control is offered of the proportions of olefins of different molecular weight and degree of unsaturation. As will be brought out at a later point, the possibility of such a control may sometimes be of advantage in view of the varying character of the aromatics with which the olefins are to be condensed in the case of particular stocks to which aromatics have been added from outside sources or in which

aromatics or benzenoid hydrocarbons are present as a result of the cracking of some heavier charging oil.

Another feature of the first step of the process of the invention appears in the use of hydrocarbon gas mixtures instead of individual hydrocarbons as starting material. When employing individual hydrocarbons, such as methane or ethane for the production of ethylene by cracking, the allowable variation in time factor if maximum yields are to be produced is only 0.0012 second either side of the optimum. When employing gas mixtures of the nature of gases from cracking, the time of heating may be varied over a considerably wider range without seriously affecting the yield.

While the first step of the process is particularly directed to the treatment of gases from cracking processes, other hydrocarbon gases may be treated such as natural gas, oil gases resulting from the intensive cracking of heavy hydrocarbons, etc. Furthermore, blends may be produced by suitable mixing of hydrocarbon gases from different sources so that improved results are obtained.

The reactions involved in the second step of the process are essentially those between olefins and aromatics and as a typical example of this type of reaction the reactions which occur between propylene and benzol in the presence of sulphuric acid at a temperature of approximately 0° C. may be cited. To produce these reactions propylene is passed into a well stirred mixture of benzol and concentrated sulphuric acid in proper proportions, the main product being mono-iso-propyl benzol according to the following reaction:



There is also produced concurrently a limited yield of di-iso-propyl benzol according to the following equation:



the relative production of the two compounds being dependent upon such factors as the relative proportion of the two hydrocarbons employed, the amount of sulphuric acid present and the exact temperature which to some extent controls the rate and course of the reaction.

Similarly condensations between butylenes, amylenes or heptylenes and benzol or its homologs may be produced with a minimum degree of polymerization occurring between the olefinic hydrocarbons. The compounds thus produced between benzol and olefins up to 5 carbon atoms wherein one molecule of olefin condenses with one molecule of benzol, boil within the ordinary range of commercial motor fuels, say below 430° F., and consequently their addition to any given gasoline to increase its anti-knock quality causes very little change in the distillation curve of the fuel. Condensation products which are of a higher boiling character, are usually formed in such small amounts that they vaporize along with the lower boiling hydrocarbons and cause no special difficulties in carburetion. If formed in larger quantities they may be left as residue in the redistillation of the products, either alone or mixed with gasoline.

The olefins produced under the special conditions of cracking characteristic of the first step

of the process may be reacted and combined with aromatic hydrocarbons in several ways, all of which alternatives are comprised within the scope of the invention though obviously the alternative methods may not be exactly equivalent in their ultimate results. In one mode of operation the olefins in the treated gas mixture may be reacted with individual aromatic hydrocarbons (or mixtures thereof) such as benzol, toluol, the xylols, etc., and the compounds formed may then be utilized as blending material to increase the anti-knock value of gasolines which are deficient in this respect. In another mode of operation which is of quite general utility, the highly olefinic gas mixtures from the first step of the process may be reacted with aromatics previously blended with gasoline so that the anti-knock derivatives of mixed paraffinic-aromatic character are produced in situ, and any further refining comprising limited sulphuric acid treatment, sweetening, steam distillation, etc., is conducted upon the mixture as a whole. In still other cases the olefinic gas mixture may be reacted with hydrocarbons of an aromatic character which are produced in the pyrolysis of naphthenic or mixed base charging oils such as distillates or residua from California or Texas fields, there being no need in certain of these cases for the addition of any large amount of aromatic hydrocarbons from outside sources to furnish material to react with the olefinic gases.

In practicing the first step of the process involving the pyrolysis of hydrocarbon gas mixtures under accurately controlled conditions of temperature, pressure and time any suitable type of apparatus may be employed since the invention is not limited to any particular modification of plant design or type of equipment. The materials used in heating elements employed in the first step will be determined to some extent by the temperatures employed, tubes of high chromium steel and other high melting alloys being utilized at the lower ranges while tubes of refractory materials such as fire clay, silica, sillimanite, etc., are best employed at the higher temperatures which approach the fusing point of iron.

The apparatus employed in the first step is preferably designed to permit accurate control of time factor and in most cases the heated reaction zone will consist of a tube of relatively small capacity through which the gas mixture is drawn at an accurately controlled rate. The tube may be heated by any suitable source of heat such as ordinary flames or hot combustion gases, or electrical resistors may be used with due consideration of the cost factor involved. The gases may be preheated before passage through the reaction zone to some point under the critical conditions necessary for best results, this preheating involving the use of ordinary tubular heating elements heated by combustion gases, care being exercised, however, that the gas mixture is not brought too soon to the temperature required for the desired reactions. The process can be carried out by alternately heating a furnace consisting of stones with canals therebetween and then passing the gas through the hot canals.

After passage through the main reaction zone, the gas mixture is preferably quickly cooled so that the time factor is accurately controlled and the decomposition reactions are stopped at a point corresponding to maximum production of desired products.

In conducting the second step of the process,

special equipment is seldom necessary, the ordinary batch and continuous sulphuric acid treating plants common to most petroleum refineries being generally adaptable to use, if means are provided for maintaining the necessary temperatures. For example, a regulated amount of cooled sulphuric acid of commercial grade may be added to an ordinary cone bottomed agitator (preferably well insulated) a regulated amount of benzol or other aromatic hydrocarbon subsequently added and the mixture agitated either by mechanical means or by circulating pumps. During the agitation or circulation of the benzol and sulphuric acid the olefinic gas mixtures from the first step may be passed therethrough at ordinary pressures, the olefinic constituents under these conditions reacting with benzol to form homologs of benzene which are of high anti-knock value and suitable for use as blending material to increase the knock rating of inferior or knocking gasolines.

In the second step of the process other refining treatment may be brought about incidental to the main reactions of condensation between olefins and aromatics when the reactions occur in gasolines containing undesirably large amounts of color and gum-forming compounds and high sulphur content such as, for example, gasolines from cracking high sulphur oils. In these cases, the acid treatment may serve to polymerize di- and tri-olefines to high boiling polymers readily removable by subsequent distillation and at the same time produce high anti-knock compounds by the union of liquid mono-olefins and aromatic or cyclic hydrocarbons according to the same general type of reaction which takes place between the olefins from the first step of the process and the aromatic hydrocarbons.

In cases involving the alternate method of treating gasoline containing aromatics with olefinic gases, the use of the process in connection with the improvement of such gasoline does not preclude the use of other refining treatments upon the gasoline either before or after the production of the condensation reactions. Thus, for example, cracked gasolines may be treated by the use of sulphuric acid, neutralized, sweetened and redistilled, after which aromatics from other sources may be added to them. After the reactions of condensation have been produced in the gasoline or the condensation products separately produced have been added to the gasoline, the blend may be further treated by reagents adapted to remove color, gum and sulphur and the treated gasoline may be rerun if it is found that the best results are obtained by this type of operation.

An example of the results obtainable by the use of the process of the invention may be given which involves in the first step the further processing of the cracking gas mixture shown in a preceding part of the specification, the temperature employed being 950° C., the pressure 50 mm. of mercury absolute and the time factor 0.0075 second. Under these conditions the percentage of acetylene in the gas mixture will be practically 0, the percentage of ethylene approximately 20 and the percentage of propylene and higher olefinic homologs 15 to 20, the other constituents being chiefly paraffin hydrocarbons which do not enter into the condensation reactions.

The gas mixture produced in the first step may be conducted into a gasoline blend consisting of 80% by volume of a straight run paraffinic gas-

oline and 20% by volume of benzol, the octane number of the blend being 60%. Sulphuric acid in an amount equal to approximately 20 pounds per barrel of the blend may be present and be maintained in suspension in a finely divided condition by means of mechanical stirring equipment or pump circulation during the admission of the olefinic gas mixture. Cooling coils are preferably employed to prevent undue temperature rise and minimize oxidation and polymerization reactions. The gas mixture may be introduced at the rate of 10 to 15 cubic feet per hour per barrel of blend and the treatment continued until the blend has increased 18% by weight, this weight increase corresponding to an increase of approximately 14% by volume of the blend.

The acid layer may be separated and removed, and the treated gasoline neutralized and redistilled to the same end point which the blend had prior to the gas treatment, there being recovered a finished gasoline equal to 110% by volume of the original blend. This gasoline may have the properties shown in the following table:

|                             |     |
|-----------------------------|-----|
| 25 Gravity °A. P. I.        | 56  |
| End point °F.               | 410 |
| Color, Saybolt              | 30  |
| Mg gum (copper dish method) | 20  |
| 30 Octane number            | 70  |

The advantages of the process are evident from a consideration of the foregoing data which indicates that an overall increase of 25 points in octane number was obtained by the combination of steps comprising the process of the invention since the straight run gasoline prior to the addition of benzol and contacting with the cracked gases was only 45%. Moreover, the overall yield apart from that obtained by the addition of benzol was increased 10%.

Neither specification nor example is to be construed in the light of imposing undue limitations upon the generally broad scope of the invention.

I claim as my invention:

1. A process for increasing the anti-knock value of gasoline containing a hydrocarbon of the benzene series, which comprises adding sulphuric acid to the gasoline, passing olefinic material in gaseous form into the resultant mixture, reacting the olefinic material with said hydrocarbon in the presence of the acid to form an alkylated aromatic having anti-knock properties, and separating the gasoline containing the thus formed alkylated aromatic from the acid layer.

2. A process for improving cracked gasoline containing, as a result of the cracking, a hydrocarbon of the benzene series, which comprises adding sulphuric acid to the gasoline, passing olefinic material in gaseous form into the resultant mixture, reacting the olefinic material with said hydrocarbon in the presence of the acid to form an alkylated aromatic having anti-knock properties, and separating the gasoline containing the thus formed alkylated aromatic from the acid layer.

3. A process for increasing the anti-knock value of gasoline containing a hydrocarbon of the benzene series, which comprises adding an alkylating agent to the gasoline, passing olefinic material in gaseous form into the resultant mixture, reacting the olefinic material with said hydrocarbon in the presence of said agent to form an alkylated aromatic having anti-knock properties, and separating the gasoline containing the thus formed alkylated aromatic from the alkylating agent.

4. A process for improving cracked gasoline containing, as a result of the cracking, a hydrocarbon of the benzene series, which comprises adding an alkylating agent to the gasoline, passing olefinic material in gaseous form into the resultant mixture, reacting the olefinic material with said hydrocarbon in the presence of said agent to form an alkylated aromatic having anti-knock properties, and separating the gasoline containing the thus formed alkylated aromatic from the alkylating agent.

VLADIMIR IPATIEFF.